

# UNITED STATES PATENT OFFICE.

GEORGE H. JOHNSON, OF PAXTON, MASSACHUSETTS.

## BLACKING FOR HEATED IRON.

No. 887,813.

Specification of Letters Patent.

Patented May 19, 1903.

Application filed December 26, 1897. Serial No. 406,188.

To all whom it may concern:

Be it known that I, GEORGE H. JOHNSON, a citizen of the United States, residing at Paxton, in the county of Worcester and State of Massachusetts, have invented a new and useful Blacking for Heated Iron, of which the following is a specification.

This invention relates to a blacking or dressing for treating iron which is intended 10 to be heated in use.

Many compositions for stove blackings and polishes have been made but most of them involve, as the principal ingredient, graphite which is applied mechanically and 15 which is not in any way united to the iron but is merely rubbed on the surface of the same so that it will present a black surface for a limited period of time. The graphite is usually put up with a binder or the like 20 which is decomposed by heat so that after the blacking or dressing is applied it will become loosened and disappear in a short time after the stove or other article on which it is used is heated to the ordinary temperatures 25 to which stoves and the like are subjected.

The principal purpose of this invention is to provide a blacking or dressing which is so affected by the ordinary heating of a stove or the like that when applied to the iron it 30 will produce a coating intimately united with the surface of the iron without the interposition of any binder or the like. In this way, a surface is secured which will only be more permanently fixed by heating and can 35 not be removed in the ordinary use of the stove except by the repeated rubbing of metal surfaces against the iron. In order to accomplish this result, the iron is dressed with a metallic salt in solution either in combination with other substances or not, said salt being of such nature that a black metallic oxid having a metallic luster will be fixed to the surface of the iron when the stove is heated. Preferably also a metallic salt is 40 used which is of such a nature that the desired result may be secured in two ways; first simply by decomposing the salt when the stove is heated to produce the black oxid; and second, by precipitating a metal 45 from the salt upon its contact with the iron even in a cold state and leaving the metal intimately united with the surface of the iron and in such condition that when the metal is heated the black oxid will be formed 50 and will be united with the iron as in the

other case. In all cases, the black oxid is in contact with the iron when *in statu nascendi*, so that it unites therewith and thus produces a result not attained by simply coating the iron with the black oxid in suspension in a liquid, or mixed in a paste.

As a specific example of a practicable way of carrying out the invention, cupric hydroxid is dissolved, preferably in ammonia water, and applied to the surface of the iron. It is 60 well known that this hydroxid possesses the property of losing its water when heated, even when under water and being changed to black cupric oxid; consequently, if it is applied to a hot stove the result will be the production of a surface of cupric oxid on the iron and as this surface is formed in a chemical manner while in contact with the iron which is in a heated condition, it has been found in practice that it is firmly united with the iron 65 and can only be removed by slow degrees in the ordinary use of stove. Obviously, any further heating of the stove has no effect on it after it is once fixed unless it be to more firmly fix it in position. Consequently, the 70 coating is exceedingly durable in practice and will be removed only in the course of time by the constant attrition which it receives by the use of utensils ordinarily employed on stoves. Another important advantage of this method of carrying out the 75 invention is that the cupric oxid has a metallic luster and that it is composed of a black, amorphous powder which at high temperatures settles together so as to form a hard 80 coating, which can be blacked over with ordinary forms of blacking so as to receive a high polish therefrom. It is preferred also to place a black filler of any kind, as for example, tannate of iron, in the solution in any 85 desired proportion but preferably in a small quantity. This especially when used with the nitrate solution mentioned hereinafter gives the composition a body and serves to 90 give a smoother surface to rough iron. It 95 also by means of its color makes it look more like an ordinary blacking and has no deleterious effect on the article when used for the purpose for which it is intended. Another salt which can be used is the basic copper 100 carbonate. The cupric nitrate also may be used as it is easily converted by heat into black cupric oxid and as it is readily soluble in water and alcohol. When dissolved in 105 water for this purpose, it is preferred to first 110

heat the solution almost to the boiling point and then allow it to cool. It has been found in practice that while this action does not destroy the cupric nitrate, it prevents the 5 formation of gases in the solution when the same is heated to moderate temperature, as for example, by being exposed to the sunlight, and thus makes a more stable article for commercial purposes. This composition 10 also is capable of precipitation of its copper when brought into contact with the iron in a cold state, leaving the copper united with the surface of the iron in such form that black 15 oxide will be produced when it is heated afterwards. When the tannate of iron is used the nitrate should be slightly acid, and may contain free nitric acid.

I am aware that the materials used and the 20 method of carrying out the invention may be varied by a skilled chemist without departing

from the scope of the invention as expressed in the claims.

Having thus described my invention, what I claim is:—

1. A blacking or dressing for iron surfaces 25 comprising a solution of a copper salt capable of being decomposed by heat to produce black cupric oxid.

2. A blacking or dressing composition for iron surfaces comprising a black filler, and a 30 solution of a copper salt capable of being decomposed by heat to produce black oxid of copper.

In testimony whereof I have hereunto set my hand, in the presence of two subscribing 35 witnesses.

GEORGE H. JOHNSON.

Witnesses:

A. E. FAY,  
C. F. WESSON.